

## UNITED STATES PATENT OFFICE

2,287,093

## MATCH

Carleton Ellis, Montclair, N. J., assignor to Standard Oil Development Company, a corporation of Delaware

No Drawing. Application December 9, 1939,  
Serial No. 308,391

3 Claims. (Cl. 52—25)

This invention relates to matches and specifically to compositions of matter that improve the burning properties of matches and flame transmission from the match head to the match body. It also involves employment of compositions of matter which are particularly effective in augmenting the burning and igniting qualities of matches and which contain nitrated hydrocarbons or oxygenated derivatives of nitrated hydrocarbons.

Heads of matches ordinarily contain combustibles, materials for supplying oxygen, binding agents, fillers and sometimes waterproofing compounds. Combustibles may be phosphorus, phosphorus sesqui-sulphide, antimony trisulphide or other compounds that are readily ignitable by friction. Peroxides, nitrates, chlorates and perchlorates of metals are used as sources of oxygen. Water-soluble glues or gums are used as binding agents. Fillers commonly employed are powdered glass, pumice stone, sand, chalk, plaster of Paris, pulverized asbestos, siliceous marl, kieselguhr or any absorbent material that is not materially changed during combustion of the head. Fillers slow down the speed of burning of the head and thereby allow sufficient time for the flame transmitter to operate. These materials (fillers) being inert absorb heat from the burning head.

Wood splints or cardboard strips often form the match body. Paraffin wax, stearin or sulphur are used as flame transmitters and are impregnated into the splint or cardboard strips.

In this specification, I define a filler as a material preventing too rapid a propagation of flame through the match head. A flame transmitter is a substance that aids in conveying the flame from the match head to the match body.

One object of my invention is to provide a filler composition containing a nitrated hydrocarbon, or an oxygenated derivative of a nitrated hydrocarbon, that retards too rapid progression of flame through the head and at the same time produces a hotter flame. Another object is to cause the body of the match to ignite rapidly by impregnating said body with nitrated hydrocarbons or oxygenated derivatives of nitrated hydrocarbons. Other objects will be apparent from the disclosures in this specification.

This invention is applicable to both safety matches, as well as to the ordinary strike-anywhere matches.

I have observed that the following groups of compounds, nitroparaffins, nitro mono-and polyhydroxy alcohols, nitro substituted aliphatic esters or nitro derivatives of 1,1-di(nitroalkoxy)-alkanes are especially applicable as impregnating agents for fillers or match bodies.

Nitroparaffin wax can be made by reaction of paraffin wax with nitric acid at a temperature

slightly above the melting point of the paraffin wax. If desired, a catalyst (e. g., aluminum nitrate) may be used with the acid. After reaction is finished, the wax layer is washed with water to remove the excess nitric acid. Furthermore, the nitrated wax layer can be extracted with acetone, or other appropriate solvent, in which paraffin wax exhibits only a very limited solubility and after evaporation of the solvent a solid concentrate of nitrated wax can be secured.

Nitrohydroxy compounds, suitable for my purpose, can be made by combining a nitroparaffin with an aliphatic aldehyde. Nitroalcohols or 15 nitroglycols are obtained, depending upon whether one or two moles of aldehyde, respectively, are reacted with one mole of the nitroparaffin. Reaction is carried out in the presence of an inert liquid medium, such as water, alcohol, ethylacetate, and in the presence of an alkaline catalyst, e. g., calcium hydroxide or potassium carbonate. If the reaction medium is water, then the products (after removing any insoluble material by filtration) can be isolated 20 either by extraction with a low-boiling water-immiscible solvent followed by evaporation of the solvent, or by chilling the aqueous medium and thereby effecting crystallization of the desired material. In case the liquid medium is non-aqueous, after removal of insoluble material it may be eliminated by distillation and the residue then subjected to an extraction operation or to a recrystallization step, as the case may be.

Esters of the nitroalcohols or of nitroglycols 30 are obtained by interaction of the nitrohydroxy compound with an acid anhydride. Catalysts, such as hydrogen chloride, are useful in some cases. The product is isolated by pouring the reaction mixture into a water solution of an alkali, whereby the ester separates as a water-insoluble layer and any unreacted acid anhydride (or acid) is neutralized.

Aldehydes, such as paraldehyde or paraformaldehyde, in ether solution combine with nitroalcohols or nitroglycols (in the presence of hydrogen chloride, for example) to furnish acetals or formals, respectively. In most instances, molecular proportions of the reacting compounds are used. The ether is evaporated from the solution, and the resulting formal or acetal (obtained as a residue) washed with water. The acetals and formals are classed as 1,1-di(nitroalkoxy)-alkanes.

I have observed that a non-combustible absorbent material impregnated with one or more of the nitro derivatives of the group consisting of nitroparaffins, nitrohydroxy alcohols, nitro substituted aliphatic esters or nitro substituted 55 1,1-di(nitroalkoxy)-alkanes forms a flame retarder superior to an unimpregnated filler. The

treated flame retarder is equally as efficient (as the untreated one) in slowing down the flame propagation but at the same time helps produce a hotter flame which ignites the flame transmitter and match body more easily.

Impregnation of the filler by the nitro compound or compounds may take place by simple mixing. This method is applicable to solid nitro bodies that can be liquefied (by mild heating) without decomposition and to low or high-boiling liquids. Best results are obtained by adding the material to be absorbed slowly to the filler with continuous mixing.

When the impregnating agent is a solid, not readily liquefied, a solution of it may be incorporated with the filler. It is preferable to use a low-boiling solvent that can be removed readily by mild heating or by spontaneous evaporation at room temperature. The method of mixing the solution with the absorbent may be similar to that described previously when a liquid nitro compound was the impregnating material.

Other methods commonly used for absorbing one material on another may be employed, in certain instances, where the previously mentioned procedures do not give the desired result, an example being distillation of an ordinarily solid or liquid compound and absorbing the vapors on a porous body, which would be suitable as a filler. Distillation may be effected at atmospheric or sub-atmospheric pressure as may be necessary with the particular compound employed. In some cases it may be desirable to treat the absorbent material with vapors under super-atmospheric pressure.

By proper choice of absorbents, the more volatile nitro compounds can be used and the resulting composition will be stable. Although very little of even the volatile nitrated derivatives are lost by evaporation from the filler, when the match head ignites, the impregnating agents are readily released and thereby become available to burn and supply extra heat to the burning head. The extra heat thus produced ignites the flame transmitter and match body more readily than when an untreated filler is employed.

Match head compositions superior to ordinary match head mixtures can be made by substituting, in part or in whole, an impregnated filler for an untreated one.

The same compounds may be used for flame transmission as have been described for impregnating fillers. The body of the match may be impregnated by dipping into a liquid or molten nitro compound or a solution thereof in a volatile solvent. When treating splints or cardboard strips, it is important to have a very fluid impregnating bath. The desired consistency may be gained by controlling the temperature or by using mixtures of nitro compounds or mixtures of nitro compounds and ordinary impregnating agents (e. g., paraffin wax or stearin). In some instances, a solvent, in minor proportion, may be employed to control viscosity of the impregnating mixture. In the last named case, a drying period should be allowed before the head is put on the splint. When the nitro compounds are melted before application, the treated match bodies should be cooled to the point where the impregnating compound becomes solid before the head is applied.

Solid compounds that decompose on heating or have too high a melting point may be dissolved in an appropriate solvent and this solution used

for impregnating the splints. Solvents having a low-boiling point best serve this purpose. A concentrated solution is most desirable and, consequently, solvents that will dissolve a considerable quantity of nitro compound in a small volume of solution are preferred.

Mixtures of nitro compounds or of nitro compounds with ordinary flame transmitters (e. g., paraffin wax or stearin) can be dissolved in a solvent or in a mixture of solvents and the solution used as in the preceding manner. In any case, where a solvent is employed, it is preferable to evaporate the latter from the treated match body before the head is attached.

I have observed that nitroparaffin wax behaves quite differently from paraffin wax on a burning splint or cardboard strip. As the molten wax precedes the flame along the splint, it has a tendency to be absorbed by the match body. Nitroparaffin wax is not absorbed as rapidly as paraffin wax and, consequently, if the same quantity of both waxes is impregnated into two match splints, the nitro wax will travel farther down the burning splint than the paraffin wax.

The main object of impregnating splints with flame transmitters is to facilitate ignition of the match body. Therefore, the nitroparaffin wax is more efficient because its flame transmitting power extends farther down the splint. Another explanation of this increased efficiency is that less nitro wax is necessary to propagate flame along a given length of stick than when paraffin wax is used.

35 Splints treated with nitroparaffin wax ignite more readily than those treated with paraffin wax. Match bodies which are not impregnated do not become ignited as easily as splints treated with nitro compounds.

40 The following examples will illustrate more clearly my invention. I do not wish my invention to be limited only to the specific compounds named therein, to the proportions of ingredients mentioned or to methods described.

Example 1.—A nitroalcohol, 2-nitropropanol, was made by the following method. One mole of nitroethane was mixed with an equal volume of water. To the water-nitroparaffin mixture 0.5% of calcium hydroxide (based on the weight of nitroparaffin) was added. The whole mixture was stirred vigorously while one mole of formaldehyde in a water solution was added. Afterwards, the nitroalcohol from the combination of the aldehyde and nitroparaffin was extracted with ethyl ether. The latter was evaporated under reduced pressure and the nitroalcohol, 2-nitropropanol obtained as a residue.

Example 2.—Twenty parts of 2-nitropropanol, as made in Example 1, were admixed with 80 parts of infusorial earth. This alcohol is a liquid and can be added in small portions to the filler. Each addition of the alcohol was thoroughly incorporated with the filler. The treated filler was used in a match head having the following formula.

|                                                     | Parts |
|-----------------------------------------------------|-------|
| KClO <sub>3</sub> -----                             | 450   |
| K <sub>2</sub> Cr <sub>2</sub> O <sub>7</sub> ----- | 100   |
| Treated filler -----                                | 100   |
| Flowers of sulfur -----                             | 60    |
| Amorphous phosphorus -----                          | 10    |
| Gum arabic -----                                    | 140   |
| Water ----- (*)                                     |       |

\*Enough to give desired consistency.

The glue was dissolved in a small amount of water, and pulverized potassium chlorate and potassium dichromate were incorporated. After each compound was added, sufficient water was admixed to keep the mixture in a pasty form that could be easily and safely handled. The filler, flowers of sulfur and phosphorus were incorporated in the order named. The final mixture had the consistency of thick paint. Wood splints were used in making matches with this match head composition. The splints were dipped into the head mixture and then dried. These match heads ignited the splints better than a similar head composition containing an untreated filler.

*Example 3.*—To make the acetal of 2-nitro-2-propyl-propanediol-1,3 the following procedure was employed. Two moles of formaldehyde were reacted with one mole of 1-nitrobutane in the manner described in Example 1. The resulting nitroglycol was extracted with ethyl ether and the ether evaporated. Two moles of paraldehyde were combined with 3 moles of 2-nitro-2-propylpropanediol-1,3 using dry hydrogen chloride as a catalyst and ethyl ether as the liquid medium. The mixture was allowed to react over night, and again dry hydrogen chloride added. After standing for several more days, the reaction mixture was washed with water (to remove hydrogen chloride and unreacted material) and dried. Evaporation of the ether under reduced pressure, yielded the acetal as an almost colorless solid.

*Example 4.*—Two parts of acetal of 2-nitro-2-propylpropanediol-1,3 were dissolved in four parts of ethyl ether. The solution of the solid glycol was mixed with four parts infusorial earth. The solvent was allowed to evaporate and the residual product used in the same formula as in Example 2. The matches obtained from this match head composition were superior to similar matches made with untreated fillers in that after striking they ignited splints more readily. The head flamed smoothly and burned with a hotter flame than when an ordinary filler, e. g., kieselguhr or powdered glass, was used.

*Example 5.*—Nitrated paraffin wax was prepared in the following manner: Ten parts of the wax were admixed with 12.2 parts of hydrated aluminum nitrate ( $Al(NO_3)_3 \cdot 9H_2O$ ) as catalyst, and after the mixture was heated to 100° C. then 4.3 parts of nitric acid (sp. gr. 1.42) were added. The reactants were kept at 100° C. for 25 hours, during which time they were vigorously stirred. Also during this period, at approximately 6 hour intervals, there were added 4.3 parts, 4.3 parts and 2.1 parts of nitric acid. The waxy layer was withdrawn, washed well with water to eliminate any entrained acid or catalyst, and then extracted with acetone. After filtering any insoluble material, evaporation of the solvent (acetone) yielded a concentrate of nitrated wax.

*Example 6.*—Nitroparaffin wax, as made in Example 5, was melted and heated to 100° C. Wood splints were immersed therein to the extent of approximately three-eighths of an inch, withdrawn and the nitrated wax allowed to harden. Heads similar in composition to those described in Example 4 were put on the impregnated splints. These matches were easy to ignite and because the nitro wax is not absorbed into the burning splint as rapidly as ordinary wax, they were superior in burning qualities to matches made from splints treated with ordinary paraffin wax.

*Example 7.*—The formal of 2-nitro-2-methylpropanediol-1,3 was prepared according to the procedure given in Example 3, with the exception that paraformaldehyde was substituted for paraaldehyde.

*Example 8.*—Splints were treated with the formal of 2-nitro-2-methylpropanediol-1,3 by dipping into the compound, which is a liquid at ordinary temperature. A short time is allowed for the formal to be absorbed by the splint and then a head similar in composition to that described in Example 4 was put onto the match body. The matches, when dry, ignited easily and much more readily than when untreated splints were used.

*Example 9.*—An ester of 2-nitro-2-methylpropanol and acetic acid was made according to the following directions. The alcohol was obtained by condensing formaldehyde with 2-nitropropane as in Example 1. Molecular proportions of the nitroalcohol and acetic anhydride (plus 10% excess) were mixed together. Dry hydrogen chloride was passed through the solution for a short time and then the reaction was allowed to proceed at room temperature for three or four days. Afterwards, the reaction mixture was poured into a sodium bicarbonate solution to neutralize the excess and unreacted anhydride. The acetate separated from the aqueous solution as an insoluble layer and this was withdrawn, washed with water and dried.

*Example 10.*—The acetate of 2-nitro-2-methylpropanol from Example 9 is a liquid. Splints were dipped into the acetate to a depth of three-eighths of an inch, and a few minutes time was allowed for the liquid to be absorbed into the stick. Heads similar in composition to Example 4 were put onto the splints. The matches were dried and when struck, the matches with treated splints became ignited easier than when no treatment was applied to the sticks.

*Example 11.*—One part by weight of the acetal of 2-nitro-2-propylpropanediol-1,3, as obtained in Example 3, was dissolved in an equal part of ethyl ether. Splints were dipped into the acetal solution and then gently heated to evaporate the ether. The impregnated splints afterwards were dipped into a match head composition similar to that described in Example 4. The matches, after the head was dried, ignited easily and much better than when the match body was untreated.

It will be seen from the foregoing disclosures that my invention provides matches with improved burning and igniting qualities. It also involves inert and non-combustible flame retarders or fillers which are impregnated with nitro compounds which in turn aid in prolonging or extending the burning period when the match head is ignited by friction. The proportion of filler in the match head composition may vary within rather wide limits, say from about 10 per cent to about 40 per cent. Whatever the proportion employed, it should be sufficient to retard flame progression (on ignition of the match head) and thereby allow the match body (splint, cardboard strip or other combustible material) to become ignited.

Likewise, the proportion of nitro compounds may vary between wide limits. In the examples, I have illustrated filler compositions in which the proportion of nitro bodies was one-half to one-fourth that of the inert and non-combustible filler. I do not wish to be limited to these, since greater or lesser proportions may serve equally well in some instances. The quantity of nitro derivative may be as low as 10 per cent of the

inert filler and the resulting composition still function. What is necessary is that a sufficient quantity of the nitro body should be present that it will extend or prolong the initial flame period (after striking the match head) so that the flame transmitter will ignite and in turn kindle the match body.

Those nitro compounds particularly suitable for my invention include not only those aliphatic derivatives obtained by direct nitration or treatment with nitric acid, but also those resulting from the condensation of nitroparaffins with aliphatic aldehydes. The compounds prepared in this manner contain not only a nitro group, but also a hydroxyl group. Moreover, aliphatic carboxylic esters or aliphatic alkoxy derivatives of these nitrohydroxy compounds are suitable for the purpose.

My invention embraces not only match-head containing fillers impregnated with the above-mentioned nitro compounds, but also match bodies impregnated with such. In this manner, I secure not only greatly enhanced flame transmission from the match head to the match body but also superior burning qualities in the match body.

It is understood, of course, that not only are individual nitro compounds or their oxygen-containing derivatives (as mentioned above) included in this invention, but also various mixtures of such substances.

Of course, it is possible likewise to dip the finger-holding part of the splint into a solution which will prevent combustion beyond a certain point. I have found silicated soda suitable for the purpose, but other products of a similar nature may be used to reduce combustion at the

finger-holding end so that the fingers will not get burned when the match is held for too long a time after ignition.

What I claim is:

5 1. A friction-ignitable match comprising a match head consisting of a friction-ignitable composition attached to a combustible match body impregnated with a nitroparaffin containing at least one nitro group in which the nitrogen atom is directly attached to a carbon atom, the proportion of said nitro compound on said body being sufficient to transmit the flame to said match body from said match head when ignited.

10 2. A friction-ignitable match comprising a match head ignitable by friction attached to a match body impregnated for at least a portion of its length with a nitro compound containing at least one nitro group in which the nitrogen atom is directly attached to a carbon atom in a paraffinic hydrocarbon group, said nitro compound being selected from the group consisting of nitroparaffins, nitrohydroxy-paraffins, aliphatic monocarboxylic esters of nitrohydroxy-paraffins, and nitroalkoxy-paraffins, the proportion of said nitro compound on said body being sufficient to prolong burning of the match when ignited.

15 3. A friction-ignitable match comprising a match head consisting of a friction-ignitable composition in which is incorporated an inert and non-combustible filler impregnated with a nitroparaffin containing at least one nitro group in which the nitrogen atom is directly attached to a carbon atom, the proportion of said nitro-paraffin being sufficient to prolong burning of said match when ignited, and a combustible match body attached to said match head.

CARLETON ELLIS.